

## UNITED STATES PATENT OFFICE

2,497,540

FLUXES FOR THE TREATMENT OF  
LIGHT ALLOYS

Edward Frederick Emley, Clifton Junction, near  
Manchester, England, assignor to Magnesium  
Elektron Limited, London, England, a British  
company

No Drawing. Application August 26, 1947. Serial  
No. 770,763. In Great Britain August 29, 1946

2 Claims. (Cl. 75—67)

1

This invention relates to fluxes for the treatment of light alloys consisting of magnesium base alloys containing rare earth metals, and aluminium base alloys containing rare earth metals.

In the treatment of such alloys with fluxes containing magnesium chloride it has been found that more or less considerable losses of the rare earth metals occur as a result of reaction with the magnesium chloride, particularly when using an inspissated or refining type of flux which requires to be stirred thoroughly into the metal. I have accordingly endeavoured to develop an inspissated type of flux which contains substantially no magnesium chloride. For this purpose I have endeavoured to develop a flux which contains a mixture of chlorides (which I term a protective base) having a sufficiently low melting point to enable the flux to prevent burning of the metal and to provide, together with a sufficient quantity of inspissating agents, to enable the flux to have the required viscosity, a pasty viscous covering on the metal. In other words I have endeavoured to inspissate a mixture of chlorides not containing magnesium chloride in a manner in which it has previously been proposed to inspissate chloride mixtures consisting largely of magnesium chloride. I have, however, found that the inspissation of chloride mixtures not containing magnesium chloride is accompanied by certain difficulties. For example, attempts to inspissate a chloride mixture solely by means of an addition of magnesia, result in a tendency to liquation and "dry top" effects, that is to say the flux cover on top of the molten metal is too dry near to its upper surface, and appears to consist mainly of magnesia insufficiently wetted by the chlorides. These difficulties are apparently due to the poor wetting capacity for MgO of chloride mixtures not containing magnesium chloride.

These difficulties can be overcome by prefusing the magnesia with the chloride mixture but this results in a flux, the composition of which must be adjusted somewhat critically to achieve the required degree of inspissation, and which is barely satisfactory in its ability to extinguish burning magnesium.

Accordingly I have attempted to inspissate these chloride mixtures with calcium fluoride. The composition of these fluxes appeared to be very critical in so far as compositions tending to be somewhat fluid showed the pronounced non-wetting effects to be expected in the absence of magnesium chloride, whereas attempts to

2

overcome this difficulty by increasing the amount of the calcium fluoride until the flux was so viscous as to be incapable of showing non-wetting characteristics produced fluxes which were too dry for satisfactory protection of the metal against oxidation. The range of composition between fluxes showing the non-wetting tendency and those which are too dry is too narrow for satisfactory commercial production of such fluxes and moreover the optimum calcium fluoride content varies with temperature of the metal under treatment.

Attempts to use calcium fluoride and magnesia together gave fluxes possessing to some extent the disadvantages associated with the separate use of both these inspissating agents.

The use of strontium and barium fluorides also produced disadvantages similar to those accompanying the use of calcium fluoride.

The use of sodium and potassium fluoride gives rise to introduction of small amounts of sodium and traces of potassium into the metal both of which are objectionable, in addition to non-wetting difficulties.

The use of magnesium fluoride was initially considered impracticable, not only because it is more costly than any of the fluorides above mentioned, but more particularly because it is well known that magnesium fluoride will react with the rare earth metals in the same way as magnesium chloride.

I have now made the surprising discovery that unlike the fluorides of sodium, potassium, calcium, strontium, or barium, magnesium fluoride is substantially insoluble in certain chloride mixtures not containing magnesium chloride and I have used this discovery to make fluxes which are very satisfactory for use with alloys containing rare earth metals. I inspissate such chloride mixtures with magnesium fluoride and because the latter is practically insoluble in the chloride mixtures non-wetting does not arise. Furthermore, when the flux melts the particles of magnesium fluoride are readily wetted and coated with the protective base in which they do not dissolve and the magnesium fluoride is thereby protected from contact with the rare earth metals in the alloy and so does not react therewith.

The flux may, however, contain a minor portion of inspissating agents other than magnesium fluoride. Some small amount of magnesium chloride may be tolerated in the flux but this should not exceed 2% and is preferably less than 0.5%.

According to the present invention therefore,

a flux suitable for the treatment of the aforesaid light alloys is substantially free from magnesium chloride and consists essentially of at least two chlorides of the alkali metals and alkaline earth metals, other than magnesium, these chlorides in the absence of inspissating agents have a liquidus temperature not greater than 610° C., the flux also containing a sufficient quantity of one or more inspissating agents to enable the flux to provide a pasty viscous covering on the molten metal, and at least 75% of the inspissating agents consisting of magnesium fluoride.

I find in particular that mixtures of calcium, potassium, and sodium chlorides are suitable for inspissation by magnesium fluoride especially in the following percentages of the chloride mixture(s):

|                    | Per cent |    |
|--------------------|----------|----|
| Calcium chloride   | 40-70    | 20 |
| Potassium chloride | 6-30     |    |
| Sodium chloride    | 24-40    |    |

Some proportions of barium and strontium chlorides, (e. g. up to about ten or fifteen per cent together) of the total inspissated flux may also be included. The flux may contain (in the absence of barium and/or strontium fluorides) less than 25 per cent of barium chloride, or of the equivalent quantity of strontium chloride, or mixture of barium and strontium chlorides, reckoning 1 per cent strontium chloride as equivalent to 0.7 per cent barium chloride.

Examples of inspissated flux compositions which we have found satisfactory are as follows:

|                   |    |      |      |    |
|-------------------|----|------|------|----|
| CaCl <sub>2</sub> | 41 | 25.5 | 49   |    |
| NaCl              | 26 | —    | 23.5 |    |
| KCl               | 9  | 47   | —    |    |
| BaCl <sub>2</sub> | —  | 7.5  | —    |    |
| SrCl <sub>2</sub> | —  | —    | 7.5  | 40 |
| MgF <sub>2</sub>  | 24 | 20   | 20   |    |

In these examples the figures indicate percentages by weight of the compositions.

Magnesium base alloys containing one or more rare earth metals can be treated with fluxes made in accordance with the invention with regular production of finished alloys having at least equal freedom from traces of chloride contamina-

tion as commonly produced magnesium base alloys containing aluminium.

I claim:

1. An inspissated flux suitable for the treatment of magnesium alloys containing a rare earth metal, which flux is substantially free from magnesium chloride and consists of at least two chlorides of the alkali metals and alkaline earth metals, other than magnesium, which chlorides when in mixture alone have a liquidus temperature not greater than 610° C., the balance of the flux being a quantity of inspissating agent such as to provide a pasty viscous covering on the molten metal, and at least 75% of the inspissating agent consisting of magnesium fluoride, the quantity of magnesium fluoride being about 20% by weight of the flux.

2. A flux as claimed in claim 1 wherein the chlorides consist of the chlorides of calcium, potassium and sodium, in the following percentages of the total chloride mixture:

|                    | Per cent | Per cent |
|--------------------|----------|----------|
| Calcium chloride   | 40-70    |          |
| Potassium chloride | 6-30     |          |
| Sodium chloride    | 24-40    |          |

EDWARD FREDERICK EMLEY.

#### REFERENCES CITED

30 The following references are of record in the file of this patent:

#### UNITED STATES PATENTS

| Number    | Name            | Date          |
|-----------|-----------------|---------------|
| 2,121,292 | Haughton et al. | June 21, 1938 |
| 2,327,065 | Reimers         | Aug. 17, 1943 |
| 2,396,604 | Reimers         | Mar. 12, 1946 |

#### FOREIGN PATENTS

| Number  | Country       | Date         |
|---------|---------------|--------------|
| 342,586 | Great Britain | Feb. 5, 1931 |
| 403,891 | Great Britain | Jan. 4, 1934 |
| 489,700 | Great Britain | Aug. 6, 1938 |

#### OTHER REFERENCES

Marande, Materials and Methods, February 1946, pp. 418-424.